

June 24, 1930.

A. L. DAVIS

1,767,653

METAL ARTICLE

Filed Nov. 18, 1925

Fig. 1.



Fig. 2.



Inventor  
Alvan L. Davis  
By his Attorneys  
Phelps, Sawyer, Rice & Keen

## UNITED STATES PATENT OFFICE

ALVAN L. DAVIS, OF WATERBURY, CONNECTICUT, ASSIGNOR TO SCOVILL MANUFACTURING COMPANY, OF WATERBURY, CONNECTICUT, A CORPORATION OF CONNECTICUT

## METAL ARTICLE

Application filed November 18, 1925. Serial No. 69,812.

This invention relates to certain improvements in metal articles comprising a stem having an enlarged head thereon, and more specifically to such metal articles as cap screws or bolts.

According to an approved practice of manufacturing cap screws or bolts, cold drawn wire stock is upset to form a headed blank and the head of the blank is then shaped to be engaged by a tool, as for example, by cutting facets thereon. Cap screws or bolts so formed, however, are frequently characterized by a brittleness of the metal in the head which renders the head liable to break.

It is the object of the present invention to produce a metal article such as a bolt or cap screw, or, more generally speaking, an article consisting of a headed stem formed from cold drawn metal, such that this brittleness of the head is avoided.

With this object in view, the invention consists in the article having the characteristics herein described and specifically pointed out.

Referring to the accompanying drawings, Figure 1 diagrammatically represents, in section, a blank for a cap screw formed from a cold drawn steel wire or rod having a head formed thereon by cold upsetting; and,

Figure 2 diagrammatically represents, in section, a completed cap screw made in accordance with the invention.

Referring to the drawings, 11 represents the stem of the blank which is formed from cold drawn rod or wire and 12 represents the head. The cold drawing process has modified the original characteristics of the metal in the stem, the crystals having been somewhat elongated. In the natural condition of the metal and before the cold drawing process, the crystals in the metal from which the wire or rod is formed, are substantially equiaxed, i. e. under the microscope, they appear to be more or less cubical in form. The cold drawing, however, tends to elongate the crystals or grains in the direction of the drawing, and this is represented in Figs. 1 and 2 by the character +. A stem which has the grains or crystals in

this elongated condition is stronger, particularly as to tensile strength, than is a stem the metal in which has the crystals in normal condition.

Referring to Fig. 1, and particularly to the head, as a result of the upsetting process the form of the crystals or grains in the major part of the head has been changed so that the crystals are flattened, the metal crystals presenting a sort of laminated or schistose structure which is indicated in Fig. 1 by the character -. The structure of the stem extends somewhat up into the head, as the drawing indicates, and may form, roughly speaking, a sort of cone, and there also may be formed a somewhat smaller cone, but inverted, formed in the top of the head, the metal in these cones not being characterized by this laminated or schistose structure. In cold upsetting the head, however, the bulk of the metal in it has been converted into this laminated or schistose condition with the result that the head is brittle and is liable to break in use.

Referring to Fig. 2, the completed cap screw comprises the stem 13 and head 14. In this completed cap screw of the present invention the bulk of the grains in the metal in the head 14 are recrystallized so that they more nearly approach an equiaxed condition. As a result the head is tough and not brittle. This condition is indicated by the character O.

In forming this novel article, the head is subjected to an annealing process which should be conducted in such a way that the metal in the head is substantially annealed before sufficient heat is conducted from the head into the stem to change the characteristics of the metal in the stem. This annealing may be accomplished by subjecting the head of the bolt to a lead bath as described in my companion application Serial No. 69,813, filed of even date herewith, or it may be accomplished electrically, as set forth in the application of Morris H. Bennett, Serial No. 69,924, filed of even date herewith. As disclosed in my copending application referred to, for a bolt blank formed from cold drawn steel stock and with a cold upset head

thereon, the temperature to which the head is raised will vary according to the character of the metal but will be sufficient to relieve the stresses and strains which have been set up in the metal by the cold upsetting. The temperature will usually vary within what is known as the annealing range, that is, from around 1300° F. to around 1700° F. In annealing by a lead bath the head may be lowered into the bath until about  $\frac{7}{8}$  of the head is immersed and retained until the head is given a red heat without raising the remainder of the blank beyond a black heat. The bath should be at such a temperature and the blank should be immersed for such a period of time that the head will be heated to a temperature within the annealing range referred to without sufficient heat being conducted to the stem to change substantially its characteristics.

As disclosed in the Bennett application referred to, for a bolt blank having a stem about  $\frac{3}{8}$ " in diameter and a head about  $\frac{5}{8}$ " in diameter, a three-phase current having a voltage between electrodes of 1.3 and a current of 1100 amperes per phase, has been found suitable, the time of heating being approximately three seconds.

The result of this annealing process is to recrystallize the bulk of the grains in the metal in the head so that they are no longer in a laminated or schistose condition but more nearly approach an equiaxed condition. This annealing or recrystallization of the grains strengthens or toughens the head and removes the condition of brittleness.

Where the completed cap screw of the invention is further shaped by cold working, as for instance, where facets have been formed thereon, the metal in the surface of the facets, and, to some extent behind this surface, has its grains or crystals elongated to approach the condition of the metal in the stem. This shaping may be accomplished, for example, by the drawing operation described in my companion application, Serial No. 69,813, filed of even date herewith. This condition of reconversion or re-to by a wrench or other tool used in driving by the character X.

The result of the various operations which have been described is the production of a cap screw or similar article having a strong stem, a tough head and facets (or other outer surface) of such characteristics that they will withstand, without deformation, any ordinary amount of force applied thereto by a wrench or other tool used in driving the screw home.

The method of producing the article herein described is claimed in the said companion application, Serial No. 69,813.

What I claim is:

65 1. A cap screw or bolt having a faceted

head and a stem, the crystalline structure of the metal in the stem being modified so that some or all of the crystals are somewhat elongated whereby the strength of the stem is increased, the metal in and behind the facets of the head having somewhat the characteristics of the metal in the stem, and the bulk of the metal in the interior of the head being in the recrystallized condition characteristic of annealed metal.

2. A cap screw or bolt having a faceted head, the metal in the stem and in the facets having its crystals in the elongated condition produced by working cold, the bulk of the metal in the interior of the head having its crystalline structure in the condition produced by annealing.

3. A cap screw or bolt, the crystalline structure of the metal in the stem being modified so that some or all of the crystals are somewhat elongated whereby the strength of the stem is increased, the metal in and behind the surface of the head having somewhat the characteristics of the metal in the stem and the bulk of the metal in the interior of the head being in the recrystallized condition characteristic of annealed metal.

In testimony whereof, I have hereunto set my hand.

ALVAN L. DAVIS.

70

75

80

85

90

95

100

105

110

115

120

125

130

**CERTIFICATE OF CORRECTION.**

**Patent No. 1,767,653.**

**Granted June 24, 1930, to**

**ALVAN L. DAVIS.**

**It is hereby certified that error appears in the printed specification of the above numbered patent requiring correction as follows: Page 2, lines 49 and 50, strike out the words "or re- to by a wrench or other tool used in driving" and insert instead of recrystallization is indicated in the drawing; and that the said Letters Patent should be read with this correction therein that the same may conform to the record of the case in the Patent Office.**

**Signed and sealed this 2nd day of September, A. D. 1930.**

**(Seal)**

**M. J. Moore,  
Acting Commissioner of Patents.**